

Jan. 20, 1959

C. D. BARTON ET AL

2,869,944

JOURNAL BOX LUBRICATOR PAD

Filed Nov. 1, 1955



Fig. 1.



Fig. 2.

INVENTORS  
Clarence D. Barton  
BY Morris A. Case  
J. E. Rofeld  
ATTORNEY.

1

2,869,944

**JOURNAL BOX LUBRICATOR PAD**

Clarence D. Barton, Kansas City, and Morris A. Case, Parkville, Mo., assignors to Gustin-Bacon Manufacturing Company, a corporation of Missouri

Application November 1, 1955, Serial No. 544,101

5 Claims. (Cl. 308—243)

This invention relates to a journal box lubricator pad for retaining and wicking car journal lubricating oil in standard railroad journal boxes and refers more particularly to such a pad having a relatively high density outer layer and a relatively low density filler, both of fibrous mat, the filler mat being rolled upon itself to form a cylindrical core and the pad assembly having means to prevent the soft center from working out of the shell and the packing itself from shifting out of position in the journal box due to the rotary motion of the journal therein.

Standard railroad journal packing boxes completely surround a cylindrical journal having a flanged outer portion thereon. This flanged portion constricts the space between the journal and the packing box so that the entrance to the packing chamber is smaller than the space to be occupied by the packing material, thus making it necessary to bend and compress packing materials being inserted in the box. Additionally, in use, the babbitt-faced bronze bearing which overlies the journal may jump a considerable distance from its seat on the journal, as, for instance, as much as a quarter of an inch.

The prevalent form of journal box packing is cotton and wool waste material which has been immersed in and saturated with oil for a considerable period prior to use. The purpose of such journal packing is to wick up oil from the bottom of the journal box and transfer it to the underside of the journal so as to continuously lubricate the surface of the journal as it passes under the bearing. Thus, additional quantities of oil are inserted in the box, occupying various levels in the lower portion thereof and wicking up through the packing material to the underside of the journal.

Due to the considerable motion of the journal, if any of the packing material is loose and is carried up by the journal so as to intrude itself between the bearing and the journal, so-called "waste grab" occurs which generates considerable friction and heat and, if of sufficient magnitude and duration, causes the so-called "hot box." Since the materials of prior use, such as cotton, quickly carbonize, they contribute to friction and heat, thus promoting hot-boxes and wear on the journal. These conventional materials create a constant maintenance problem, it being necessary to closely inspect each journal at the R. R. division points, or every 250 miles.

It is the common practice to remove these packing materials at intervals, launder and renovate them, and return them to service. In the case of the loose fill or bulk materials, they are easily pulled from the box by means of a metallic hook, the fill material being fairly well integrated by the interentanglement of its fibers, and, in particular, by the thread stock present in the waste.

A shaped or formed material which will maintain a constant pressure on the underside of the journal, and therefore insure its lubrication, is preferred over the loose fill materials which have been used in the past.

2

However, difficulties of inserting and removing a molded wicking pad through the small opening have usually precluded the use of formed materials. Additionally, it has been previously impossible to provide a formed molded wicking pad which will retain its position in the lower portion centrally of the journal box and not shift out of position, especially if the pad has been in a condition of "cold set" in the box.

Therefore, an object of the present invention is to provide a formed or shaped journal box lubricator pad which exerts a constant pressure on the underside of the journal thereby insuring proper lubrication, said pad insertable in the journal box for long periods of time without removal or reconditioning while retaining its form and functional characteristics.

A further object of this invention is to provide a journal box packing element which may be conveniently inserted or removed through the small entrance to the journal box or journal packing chamber without the use of special tools.

A further object is to provide a formed or shaped journal box lubricator pad which will minimize "waste grab" while exerting constant pressure on the underside of the journal.

Another object of the invention is to provide a journal box lubricator pad having a dense outer layer which provides optimum wear, toughness for insertion and oil wicking and a lower density filter which exerts the least practicable amount of pressure on the underside of the journal while providing the desired surface contact, thereby permitting the journal to be run at a relatively low temperature, and providing optimum "cold set" characteristics and fast, easy, cold temperature breakaway of the pad from the journal.

Another object of the invention is to provide a journal box lubricator pad of resilient, fibrous mat, the upper portion thereof having an open mesh cloth fabric over the journal-contacting area which both lets go of the oil and helps prevent fibers from being torn loose from the packing and the underside covered by a heavy close-weave mesh cloth which will withstand the tearing action of packing irons during insertion of the packing into the journal packing chamber and provide a smooth surface which more readily slides over rough casting of box.

Another object of the present invention is to provide a journal box lubricator pad of resilient fibrous mat formed into a cylindrical packing element, said element having a relatively low density filler portion and a relatively high density outer shell portion and means cooperating therebetween to keep the soft center thereof from working out of the denser shell and also to prevent the entire element from shifting out of its desired position in the journal box.

Other and further objects of the invention will appear in the course of the following description.

In the drawings which form a part of the instant specification and are to be read in conjunction therewith, there is shown an embodiment of the invention and, in the various views, like numerals are employed to indicate like parts.

Fig. 1 is a side view with parts in section of the inventive journal box lubricator pad.

Fig. 2 is an end view of the journal box lubricator pad of Fig. 1.

Fig. 3 is a cross-sectional view of a journal box with the inventive journal box lubricator pad of Figs. 1 and 2 positioned therein and shown in end view.

The numeral 10 refers to the filler portion of the lubricator pad which is preferably a section of resilient fibrous mat rolled upon itself to form a cylindrical element. This mat is preferably of a density of the range 1.5 to 2.

pounds per cubic foot (1.7 pounds per cubic foot being optimum) and is preferably composed of 6 denier, 3 inch length nylon staple fibers bonded together with a thermosetting resinous binder such as phenolformaldehyde. Other synthetic materials such as Teflon (tetrafluoroethylene) and Dacron (condensation product of dimethylterephthalate and ethylene glycol) in like dimensions may also be employed. The binder of such a filler should be 20% (plus or minus 5%) of the weight of the finished mat. In formulation of the mat, the fibers are united with the resin binder in a lapping process (conventional in the art) wherein the fibers are laid on in continuous webs essentially horizontally. The fibers in such a process lie relatively parallel one another in the mat when the finished mat has been formed. Such a "fiberlap" mat has relatively greater strength and resists fiber pull-out more than mats wherein the fibers are randomly disposed in the mat. A mat of these specifications has best permanent resilience and easy compressibility for insertion. While having good permanent recovery, this material does not tend to create too great an upward pressure against the journal which would raise the running temperature. A filler exerting a relatively small amount of pressure on the underside of the journal will run at a lower temperature, have better "cold set" characteristics and will be more apt to be satisfactory in cold temperature breakaway action.

The numeral 11 designates the outer shell of the lubricator pad which preferably comprises a fibrous mat having a density of from 7½ to 13 pounds per cubic foot and preferably 10 to 12 pounds per cubic foot. The fibers of this outer shell mat are preferably 3. denier staple crimped nylon fibers 2½ inches in length, bonded together with a thermosetting resin such as phenolformaldehyde. Other synthetic fibers such as Teflon (tetrafluoroethylene) and Dacron (condensation product of dimethylterephthalate and ethylene glycol) in like dimensions may also be employed. In the shell mat the binder resin should be 35% plus or minus 5% by weight of the finished mat. The fibers are formed with the resin in the previously noted lapping process and thus are tied into this type of mat very closely and cannot be readily pulled out. A relatively high density of mat is required in the outer shell for wear, toughness for insertion and oil retention. At higher densities than listed the outer shell material retains oil too well and the bearing does not get sufficient oil. Where a single layer of outer shell mat is employed, the joint 15 is preferably positioned opposite the journal contact area next the bottom of the journal box.

The outer shell lower cover 12 is made up of knitted resin treated nylon mesh of a relatively close weave (1/16" mesh preferred). Cover 12 encloses all of the outer area of the pad but the contact area with the journal. The outer shell upper cover 13 is preferably made up of knitted resin treated nylon fabric of open mesh type, the fabric having oval openings preferably 3/8" x 1/4". The openings 13a are staggered in the fabric. The outer shell upper cover 13 is employed only in the area of contact of the journal packing with the journal (21) itself. The use of a heavy close-weave cloth on the underside of the journal packing will withstand the tearing action of packing irons during insertion of the element into the journal box. At 14 is shown the means for fixing the outer shell lower cover and upper cover to the outer shell, namely, by machine sewing the cover to the outer shell with nylon thread. The joint in the outer shell is shown at 15. This joint is preferably positioned at the bottom central portion of the journal packing opposite the journal contact area. The joint is closed by extension 12a of the outer shell lower cover which, in turn, is stitched to the cover 12 and underlying outer shell mat 11.

Heavy nylon cord loops 16 closed by knots 17 penetrate diametrically through the lubricator pad and serve

to prevent the filler portion 10 from working out of the cover or outer shell portion 11 and the entire journal packing assembly from rolling under the influence of the rotating journal when positioned in the journal box.

5 Two cords are preferably employed at each end of the packing element. The cords 16 preferably but not necessarily interengage one with the other at each end of the pad. In cross-section the cords are positioned at an angle from 47° to 53° from the vertical cross-sectional axis of the pad positioned properly in the journal box or, in other words the vertical angles between the cords may range from 94° to 106°. The purpose of the cross-tie cords is to prevent rolling action of the pad by its following the journal in its direction of rotation, thereby 10 moving up into the corner of the journal box. It has been found that a unitary pad, especially a pad formed in the manner of the applicant's pad, that is, by rolling a mat upon itself in cylindrical form (but without the crosstie cords), moves out of position in the journal box 15 by "walking" along on its outer surface similar to the motion of tracks on a tractor. Thus, such a pad does not slide or slip in the journal box but rolls along its own outer surface, the upper portion of it being carried by the rotary action of the journal. When the inventive 20 pad with the crossties in it attempts to cling to the rotating surface of the journal and move in the above described manner, one of the cords slackens and the other tightens up. Since the pad is restricted in height by the journal, the pull of the nylon cords 16 with tension on 25 the then prevails and the pad breaks loose from the journal.

Referring to Fig. 3, journal box 18 has a lower packing portion 19 bounded by inward extensions 20. Extending into the box 18 is journal 21, the portion shown in Fig. 3 comprising a milled portion seating upwardly 30 against bearing 22, and having a terminal flange portion which is not shown. The lubricator pad is designed to be positioned between the lower periphery of the journal and the surrounding box 18 and extend axially not less than the length of the bearing contacting the journal. 35 The pad is designed to over-occupy the space between said journal and said box, thereby maintaining contact with the face of the journal under the severest operating conditions for an extended length of time.

In the process of long term operation, the nylon mats 40 show a large number of highly advantageous characteristics. Such mats have tremendous oil retention capacity (up to 20 times their own weight after a few moments immersion) caused by opened-up fibers giving a large amount of fiber surface and the air spaces in the mat structure physically trapping the oil. The fibers themselves have excellent permanent resilience which is not materially reduced by immersion in oil, since they are not nearly as absorptive as cotton and, therefore, do not become soggy as do the latter. The fibers have good 45 oil wicking properties and therefore the journal bearing surface runs cooler. The fibers are relatively short and opened out and, if they leave the pad, leave individually and not in clumps (which latter case might cause grabs if the clumps were to lodge between the journal and bearing). There are no long fibers to wrap around and score the bearing. The small individual filaments melt 50 when trapped between the bearing and journal, and flow out as a lubricant or harmless part of the bearing surface. The nylon is a better conductor of heat than cotton and should conduct heat away from the bearing more readily. Additionally, the nylon is hydrophobic, tending to repel 55 water arising from sources such as high water, snow, ice, drippings and ice bunkers, etc.

From the foregoing it will be seen that a journal box 60 packing has been provided meeting all of the objects hereinabove set forth.

It will be understood that certain features and sub-combinations are of utility and may be employed without reference to other features and subcombinations. This is 65 contemplated by and is within the scope of the claims.

As many possible embodiments may be made of the invention without departing from the scope thereof, it is to be understood that all matter hereinabove set forth or shown in the accompanying drawings is to be interpreted as illustrative and not in a limiting sense.

Having thus described our invention, we claim:

1. A journal box lubricator pad comprising a resilient fibrous mat rolled upon itself to form a cylindrical filler portion, a resilient fibrous mat of greater density than that comprising the said filler portion enclosing at least the major portion of the side wall of said filler portion to provide an outer shell thereon, said outer shell covered with open mesh fabric, the journal contacting portion of said outer shell covered with fabric of more open mesh than the mesh of the fabric covering the non-journal contacting portion thereof and engaging means extending through the lubricator pad and engaging both the filler and shell portions thereof.

2. A journal box lubricator pad as in claim 1 wherein the filler portion fibrous mat has a density in the range 20 of .5 to 2 pounds per cubic foot.

3. A journal box lubricator pad as in claim 1 wherein the shell portion fibrous mat has a density in the range of 7½ to 13 pounds per cubic foot.

4. A journal box lubricator pad as in claim 1 wherein the outer shell and filler portion resilient mats are composed of synthetic fibers bonded together with a thermosetting resin.

5. A journal box lubricator pad as in claim 1 wherein the thermosetting resin in the resilient outer shell mat ranges from 30 to 40 percent by weight of the mat constituents and the thermosetting resin in the filler portion resilient mat ranges from 15 to 20 percent by weight of the 10 mat constituents.

References Cited in the file of this patent

UNITED STATES PATENTS

|    |           |                   |               |
|----|-----------|-------------------|---------------|
| 15 | 631,502   | Hagy              | Aug. 22, 1899 |
|    | 1,943,298 | Cunningham et al. | Jan. 16, 1934 |
|    | 2,044,248 | Keys              | June 16, 1936 |
|    | 2,264,250 | Shoemaker         | Nov. 25, 1941 |
|    | 2,713,524 | Hagy              | July 19, 1955 |

FOREIGN PATENTS

|         |         |             |
|---------|---------|-------------|
| 206,924 | Germany | May 3, 1908 |
|---------|---------|-------------|